

# UNITED STATES PATENT OFFICE.

KALMAN WARGA, OF NEW YORK, N. Y., ASSIGNOR TO THE METALLOGRAPH CORPORATION, OF NEW YORK, N. Y., A CORPORATION OF NEW YORK.

## DECORATING METAL SURFACES.

1,346,475.

Specification of Letters Patent. Patented July 13, 1920.

No Drawing.

Application filed May 27, 1919. Serial No. 300,134.

*To all whom it may concern:*

Be it known that I, KALMAN WARGA, a citizen of the United States, and a resident of New York, in the county of New York 5 and State of New York, have invented certain new and useful Improvements in Decorating Metal Surfaces, of which the following is a specification.

The present invention relates to a method 10 of decorating metal surfaces, such as aluminum, aluminum alloys or a mixture of metals, one of which is aluminum. More particularly, the invention relates to a method, whereby multi-color decorations, 15 designs, lettering, etc., are provided by printing process upon metal surfaces, containing aluminum.

The main object of the present invention 20 is to provide a method of the type mentioned, whereby the several color films are inseparably united and fixed by heat to the metallic surface.

With this and other objects in view, which 25 will more fully appear as the nature of the invention is better understood, the process consists in the several steps hereinafter recited and pointed out in the appended claims, it being understood that several changes may be made in the process, within 30 the scope of the claims, without departing from the spirit or sacrificing any of the advantages of the invention.

In practice, it has been found that, if a thin or comparatively thin film of vitreous 35 material is brought into contact with the heated surface of aluminum or of an aluminum alloy, or of a mixture of metals, one of which is aluminum, the said film will firmly adhere to the metallic surface. It 40 has also been found that, when the aluminum having the film of vitreous material applied thereto is raised to a sufficiently high temperature, a chemical reaction will occur between the oxid on the surface of the metal 45 and the overlying vitreous material, and as a result of such action and the heat to which it is subjected, such material will be vitrified and a compound formed which will act to cement the vitrified material to the 50 metal. The method, forming the subject matter of the present application for Letters Patent, is based on this chemical reaction, mineral colors being employed

which are incorporated in or mixed with fluxes or binders of or containing vitreous 55 material of predetermined melting points.

In order to make these pigment containing fluxes or binders applicable for printing processes, they must, obviously be mixed with liquid or viscous materials, so as to 60 obtain printing inks, which are applied to the metal surfaces by any preferred printing process, impressions being made by printing surfaces, to which the work is, ordinarily, successively presented. The liquid 65 or viscous materials mentioned should be volatile at low temperatures, so that they are adapted to evaporate from the mass before the actual cementing process between the fluxes or binders and the metal surface 70 begins, thereby preventing the formation of blisters, etc., in the designs.

The melting point of any given mixture of mineral color or pigment and vitreous flux or binder depends on the ratio between 75 the quantity of flux employed to the quantity of color or pigment, more particularly the greater the quantity of flux relative to the quantity of color, the lower the degree of temperature required for melting.

In carrying out the process, forming the subject matter of the present application for Letters Patent, first the printing inks are prepared in such a manner that the color with which the first impression is to 85 be made contains the highest percentage of vitreous flux or binder, the next color a somewhat lower percentage, and so on. It is preferable that the difference in melting temperature between any two colors following each other should be marked, but not 90 excessive.

That surface of the aluminum sheet or object, to which the design, lettering, etc., is to be applied, must, obviously, be smooth, 95 but should, preferably, be to some extent oxidized. Impressions are then made in succession on the surface, and the printed sheet or object placed into a kiln, in which a temperature is maintained to produce 100 melting of the color having the highest melting point. As the aluminum sheet or object and the several color films thereon are heated, first that color, which lies next to the sheet or object, melts and is fixed to 105 the aluminum without affecting the colors

above and adjacent the same. The second color is then reached, it fixing itself onto the first color that has already been cemented to the aluminum, the third and other 5 colors are then reached, in succession. After the cementing process, the aluminum sheet or object is removed from the kiln, preferably by passing it through lower and lower temperature, so as to prevent cracking, etc., 10 of the decoration.

15 The purpose of using colors of predetermined and different melting points is to prevent the colors from running one into another, as they are being fixed to the metal sheet or object.

18 What I claim is:—

1. The method of producing multi-color 20 decorations on metal articles containing aluminum, which consists in, first, applying to the metal surface a plurality of super-imposed color films containing each a mineral pigment and a vitreous binding material, the binding materials melting at different temperatures and the melting point 25 of the film in contact with the metal surface being the lowest, and, second, fixing said films by heat.

30 2. The method of producing multicolor decorations on metal articles containing aluminum, which consists in, first, printing upon the metal surface a plurality of super-imposed color films containing each a mineral pigment and a vitreous binding material, the binding materials melting at different temperatures and the melting point 35 of the film in contact with the metal surface being the lowest, and, second, fixing said films by heat.

3. The method of producing multicolor 40 decorations on metal articles containing aluminum, which consists in, first, applying to the metal surface a plurality of super-imposed color films containing each a mineral pigment and a flux, the fluxes melting 45 at different temperatures and the melting point of the film in contact with the metal surface being the lowest, and, second, fixing said films by heat.

4. The method of producing multicolor 50 decorations on metal articles containing aluminum, which consists in, first, printing upon the metal surface a plurality of super-imposed color films containing each a mineral pigment and a flux, the fluxes melting 55 at different temperatures and the melting point of the film in contact with the metal surface being the lowest, and, second, fixing said films by heat.

5. The method of producing multicolor 60 decorations on metal articles containing aluminum, which consists in, first, permitting the metal surface to oxidize and applying a plurality of super-imposed color 65 films containing each a mineral pigment and a vitreous binding material, the binding ma-

terials melting at different temperatures and the melting point of the film in contact with the metal surface being the lowest, and, second, fixing said films by heat.

6. The method of producing multicolor 70 decorations on metal articles containing aluminum, which consists in, first, permitting the metal surface to oxidize and printing a plurality of super-imposed color films containing each a mineral pigment and a 75 vitreous binding material, the binding materials melting at different temperatures and the melting point of the film in contact with the metal surface being the lowest, and, second, fixing said films by heat. 80

7. The method of producing multicolor 85 decorations on metal articles containing aluminum, which consists in, first, permitting the metal surface to oxidize and applying a plurality of super-imposed color films containing each a mineral pigment and a flux, the fluxes melting at different temperatures and the melting point of the film in contact with the metal surface being the lowest, and, second, fixing said films by heat. 90

8. The method of producing multicolor 95 decorations on metal articles containing aluminum, which consists in, first, permitting the metal surface to oxidize and printing a plurality of super-imposed color films containing each a mineral pigment and a flux, the fluxes melting at different temperatures and the melting point of the film in contact with the metal surface being the lowest, and, second, fixing said films by 100 heat.

9. The method of producing multicolor 105 decorations on metal articles containing aluminum, which consists in, first applying to the metal surface a plurality of super-imposed colored vitreous films, said films melting at different temperatures and the melting point of the film in contact with the metal surface being the lowest, and, second, fixing said films by heat. 110

10. The method of producing multicolor 115 decorations on metal articles containing aluminum, which consists in, first, printing upon the metal surface a plurality of super-imposed colored vitreous films, said films melting at different temperatures and the melting point of the film in contact with the metal surface being the lowest, and, second, fixing said films by heat.

11. The method of producing multicolor 120 decorations on metal articles containing aluminum, which consists in, first, permitting the metal surface to oxidize and applying a plurality of super-imposed colored vitreous films, said films melting at different temperatures and the melting point of the film in contact with the metal surface being the lowest, and, second, fixing said films by heat. 125

12. The method of producing multicolor 130

decorations on metal articles containing aluminum, which consists in, first, permitting the metal surface to oxidize and printing a plurality of superimposed colored 5 vitreous films, said films melting at different temperatures and the melting point of the film in contact with the metal surface

being the lowest, and, second, fixing said films by heat.

Signed at New York, in the county of 10 Bronx, and State of New York, this 26th day of May, A. D. 1919.

KALMAN WARGA.